# EUROPEAN PATENT SPECIFICATION

(11) **EP 0 037 929 B1**
(45) Date of publication and mention of the grant of the patent: **31.10.1984**
(21) Application number: 81102186.4
(22) Date of filing: 24.03.1981
(51) Int. Cl.: B05D 7/22

(54) **Tube coating method and apparatus**
Verfahren und Vorrichtung zur Beschichtung von Rohren
Procédé et appareil pour revêtir des tubes

(30) Priority: 11.04.1980 US 139380
(43) Date of publication of application: 21.10.1981
(73) Proprietor: Vetco, Inc., Ventura California (US)
(72) Inventor: Warren, David Allan, Cypress Texas 77429 (US); McCrory, Edwin Donald, Jr., Houston Texas 77079 (US)
(74) Representative: Sparing Röhl Henseler Patentanwälte

## Description

This invention relates to the internal coating of a heated tube wherein fusible particles are transported through the tube in a flow of air.

It is frequently advantageous to coat the inside of steel tubing with nonmetallic linings. Properly selected linings can protect the tube against erosion or corrosion. A coating surface which is smoother than that of the tubing itself can result in a decreased pressure drop of fluid flowing through the tube. For such a purpose materials have been used such as polypropylene, chlorinated polyether, various polyester, certain epoxy and vinyl polymers, polyethylene, polytetrafluorethylene, and nylon. These materials may be either thermoplastic of thermosetting, and are normally applied to the tube after it has been heated.

It is desirable that the internal coating be free from voids or pin holes. It also should have a uniform thickness and a smooth surface. The method used to coat the tube should be both reproducible and simple in operation.

It is known to heat and rotate the tube to be coated so that fusible particles conveyed in an air stream and injected into the tube will stick to the surface and form a coating thereover. There have been many methods, along with apparatus therefor, suggested involving this general concept of coating a tube.

According to the US-A-3 207 618 fluidized beds have been suggested as a supply source for the fusible particles from which location they are carried through the horizontally supported and rotated tube in a stream of air. This is generally a continuous flowing stream with excess particles collected at the other end. In some cases the apparatus provides a means for reversing flow through the tube from a second fluidized bed to promote uniformity of coating of the tubing.

It has been suggested to use a timed pulse of flow carrying the fluidized particles followed with the flow of particle-free air scavenging the tube.

These various methods in general require a significant excess of particle flow and/or timing of the cycle. Effectiveness of this operation requires that the timer be consistent and readily adjustable and that there be no leaks in the system whereby the timing would not represent an appropriate particle flow. A uniform, preferably thin and smooth coating, remains difficult to obtain in a consistent and reproducible manner.

Furthermore, it is known from the CH-A-455 588 to internally coat a tube, wherein a sufficient vacuum is used to explode the coating powder into the heated tube which is supported vertically. Therefore, one must wait for some discrete time for the powder to settle out on the internal surface of the tube, thereafter draining out excess material and possibly repeating the step as required for an appropriate coating thickness. The vertical position of the heated tube complicates the handling of the tube. The tube interior is connected to a vacuum tank via a valve which is closed before opening a further valve at the powder inlet of the tube so that the volume of the vacuum tank has no influence upon the flow of powder and thus no changes for different size tubes are possible.

It is the object of the present invention to provide a method and an apparatus which allow to achieve a uniform coating of a tube in a quick and efficient manner, and in a manner which is reliably reproducible despite variations which may effect the vaccum forming means.

Thus, the invention concerns a method for lining a heated tube comprising: supporting the heated tube to be internally coated; isolating a first end of said tube from the ingress of air; placing the tube interior in fluid communication with a tank via a second end of said tube; establishing a preselected vacuum in said tank and said tube by drawing air from a suction location beyond said second end of said tube; placing a charge of coating material in an unpacked condition within a charged location thereafter drawing the coating material into said tube by suddenly placing said charged location in fluid communication with said tube, and following the flow of coating material with a flow of air, which method is characterized by rotating said heated and horizontally supported tube; and drawing vacuum from a larger volume of said tank than in said tube; said volume of said tank being chosen so large relative to that of said tube, and the predetermined value of the vacuum therein so chosen that on sudden release of the air into said tube to be coated there is a sudden flow of air which is smoothly and immediately reduced to a lower vacuum level in the tube interior.

The apparatus for carrying out this method includes means for supporting the heated tube to be lined; a container for holding fusible particles which are to be delivered to said tube; a feedpipe connected to said container and sealably connectable to one end of said tube; an imperforate tank having an inlet connection and an outlet connection; a discharge pipe connectable to the second end of said tube and connected to the inlet connection of said tank; a quick-opening valve located in said feedpipe; a vacuum pump connected to the outlet connection of said tank; sensing means for sensing the level of vacuum within the heated tube; and means for quickly opening said quick-opening valve in response to said sensing means when the measured vacuum level reaches a predetermined vacuum level, which apparatus is characterized in that means for horizontally supporting and rotating said tube are provided; said tank has a volume greater than said tube and a plurality of supplementary tanks, a plurality of pipes fluidly connected each of said supplementary tanks to said imperforate tanks and means for selectively isolating each of said supplementary tanks from said imperforate tank are provided, wherein the flow area.of said feedpipe is less than the flow area of said tube.

The tube to be coated is heated, horizontally supported, and rotated in accordance with common practice. The first end of the tube to be coated is connected to a charging container with a pipe including a quick-opening valve which is closed at this time. A measured charge of the coating material is placed in the container.

The second end of the tube is connected with a pipe to a vacuum tank. A vacuum pump places the tank and the tube under vacuum. The valve is suddenly opened so that flow suddenly occurs from the container into the tube carrying the fusible particles with it. The vacuum in the tank and the tube causes a high initial flow rate which decreases with time as the vacuum is dissipated by the inflowing air. The vacuum pump may or may not be operated during this time.

An additional valve may be added between the tube and the vacuum tank so that vacuum may be drawn within the tank while the tube is being placed into position. The valve is then opened to place the tube under vacuum as well as the tank; and when the vacuum has been established at the proper level, the quick-opening valve initiates the process as described above.

By a measuring means only a predetermined quantity of fusible particles is deposited within the container. These particles are placed within the container in an unpacked condition either by using a fluidized bed or by pouring them into the chamber over a fall breaking apparatus which will permit particles to remain in a fluffed condition for sufficient time to achieve operation of the apparatus.

The plurality of vacuum tanks which may be connected to the initial tank to provide a controllable variation in the volume which is evacuated provides ability to easily manipulate the time rate of flow variation when opening the quick-opening valve.

In the following, a preferred embodiment is described in connection with the attached drawings.
Figure 1 illustrates a schematic arrangement of the apparatus including elementary controls;
Figure 2 illustrates the relationship between vacuum and time; and
Figure 3 represents the relationship between flow through the tube and time.

The tube to be coated 10 is first cleaned and preferably internally sand blasted to white metal. A primary may or may not be applied to the clean surface. This tube is then preheated to a temperature level above the melting point of the powder which will be deposited on the internal surface. The actual temperature level depends on the coating material to be used.

This tube is then placed on rolls 12 while still hot and rotated at a predetermined speed such as 100 rpm. This rotation aids circumferential distribution of the coating.

Air tight rotary connection 14 connects the first end of the tube to be coated by pipe 16 to a charging location within container 18. The pipe 16 includes a quick-opening valve 20 whereby the container may be selectively placed in fluid communication with the tube interior.

A hopper 22 contains a supply of powdered material which is to be used for coating the pipe. A predetermined weight of the fusible particles 24 are to be used to coat the interior of the tube. The desired amount of these particles for the tube to be coated are weighed in scale 26, and the selected charge is then placed within the container 18. They are located within the container at a location generally near the outlet through pipe 16 and are preferably maintained in a fluffed or unpacked condition. As illustrated, a fluidized bed is used wherein a supply of fluidizing air passes in through pipe 28 and valve 30 through bed support 32 in accordance with well-known fluidizing principles. Alternatively the material could be placed in a container gently so that it retains a fluffed condition which may be maintained so long as the container is not unduly jarred or vibrated.

An imperforate vacuum tank 34 is connected to the second end of the tube 10 with an air tight rotary coupling 38. The connecting pipe 40 between the inlet connection 42 on the imperforate tank 34 and the rotary coupling 38 may include valve 44 if certain operation as described below is required. Otherwise this valve is not required.

A vacuum pump 46 such as an air ejector is in fluid communication with the tank 34 through pipe 48 and operated to place the tank under vacuum. With valve 20 closed and valve 44 either omitted or open, the tank and the interior of pipe 10 are both placed under vacuum. Because of the low flow rate through the pipe existing while establishing a vacuum, the vacuum level in the tank and the pipe are essentially the same and may be measured by pressure sensor 50.

After the tube to be coated is placed on the rolls 10, rotatable couplings 14 and 38 are made up; and with valve 20 closed, the weighed charge is placed in tank 18. The vacuum pump 46 is operated by an air line 52; and a vacuum is drawn in the tank 34 and pipe 10. The vacuum level during this period is illustrated in Figure 2, wherein the vacuum generally increases (51); and as illustrated, it is held at a preselected level (53).

When the vacuum reaches the desired level which is a function of the tank size, the pipe diameter and length, and the coating material used, quick-opening valve 20 is opened at time 55. This may be done as soon as the vacuum reaches the desired level, and the flat portion illustrated in Figure 2 is not necessary.

With the opening of valve 20 there is a sudden flow of air into the tube 10 as shown in Figure 3 by curve 57. The vacuum in the tank decays as illustrated by 59 in Figure 2. Accordingly, there is a sudden surge of air flow which then uniformly decreases. The sudden change in the particle environment from atmospheric pressure to the low pressure causes an explosion-like action which creates a cloud of powder which is conveyed through the tube. The rate of air flow peaks and decays in a manner related to the vacuum. Curve 59 shows the continuing air flow when the vacuum pump continues running.

The air flow pattern is a function of the tank volume and the tube size as well as the vacuum level. Some experimentation is at present required in order to determine the appropriate parameters for a particular tube and tube coating. For a particular coating too low, a tube temperature results in a considerable amount of the particles passing completely through the tube, poor adhesion, and a tendency for a powdery deposit. Any deposit also tends to be thin on the upstream end. On the other hand, too high a tube temperature not only involves handling tubes at unnecessarily high temperature levels and a waste of energy but also results in excessive coating at the upstream end of the tube.

A roughened internal surface seems to occur when the tube is too hot or when the powder is insufficiently fluffed in container 18.

Insufficient coating at the upstream end seems to be caused by too high a vacuum.

Insufficient coating at the downstream end tends to be caused by insufficient powder quantity or by too low a vacuum.

Inordinate wastage of material carried through the tube seems to be caused by too cool a tube.

Speculation on the reasons for the good results obtained in laboratory tests suggests that the result may be related to heat transfer requirements between the particles and the tube itself. High velocity is initially used when the incoming particles are radiantly exposed to the hot tubing whereby some stick at the upstream end and others are heated as they pass down the tube. The decreased flow with time retards those particles which have already passed to locations near the outlet, and the flow is reduced at a time when the particles within the dust cloud radiate not to the wall directly but to other particles which have already formed a portion of the surface. These particles, accordingly, radiate to a lower temperature level; and more time is required for heat transfer. The decreased air flow accommodates this need, and a uniform coating is obtained with little wastage.

The pipe 16 should be of a smaller diameter than the tube to be coated. This increases the velocity thru pipe 16 decreasing or avoiding the possibility of powder remaining in this pipe. Material left behind would cause erratic quantity delivery to the successive pipes being coated. The high velocity in pipe 16 as compared to the decreased velocity in the tube -10 results in good dispersal of the material with the tube.

Any particles which are carried through the system are collected in centrifugal vacuum tank 34 or in bag filter 54. These particles may be intermittently removed through valves 56 and 58, respectively. While these particles may be recycled for use, it still is not desirable to have a substantial amount of particles passing through the pipe. To the extent that there is large wastage at the pipe discharge, this provides an increasingly sizable percentage of the injected material which is passing completely through the pipe and not being deposited on the surface. The larger this amount the more variation there is in the actual pipe coating with variations in system operation.

Auxiliary vacuum tanks 60 and 62 are isola- tably connected to the vacuum tank 34 through valves 64 and 66. These tanks may be cut in or out as desired thereby varying the volumetric capacity of the vacuum system. Accordingly, the time flow characteristic of the system may be adjusted.

The system may be automatically operated with pressure sensor 50 sending a control signal through control line 68 to a set point 70 where the signal is compared to a desired pressure level signal or set point 72. This may operate to maintain a vacuum level in the tank by varying the air flow through line 52 by modulating control valve 74 with controller 76. In the event that the preselected vacuum level is reached within the vacuum tank before the remainder of the system is prepared, this control will limit the vacuum and hold it at a preselected level.

The control signal indicative of pressure level from pressure sensor 50 also passes through control line 78 to set point location 80 where it is compared with a set point 82 which represents the desired pressure level at which the quick-opening valve 20 is to open. When the vacuum reaches the preselected level, a signal is sent through control line 84 to controller 86 which opens the quick-opening valve 20.

Depending on the characteristics of the particular vacuum pump 46 being used, it may be advantageous at times to include valve 44 which may be closed while pipe 10 is being changed. The vacuum pump may operate at this time to establish a vacuum in tank 34 while the pipe is being changed. When the new pipe is in place, valve 44 is opened with pipe 10 being evacuated at which time it would be ready to operate in accordance with the above-described procedure.

Experiments were carried out to internally coat pipe to a thickness of 20 to 23 micrometers. The pipe was a range 2 drill pipe which is a pipe approximately 9.5 meters long. The material used to coat the pipe was an epoxy melt mix of approximately the following composition: The particular material used was an epoxy powder prepared by Whittaker Coatings and Chemicals Co. of Colton, California, using the trade name, "Interior Oil Pipe Coatings-E. S. Powder". The manufacturer code identifi-. cation was 8502-B235.

Four different pipe sizes were tried, and the preferred quantities of powder, vacuum and pipe temperature are set forth in Table 1. The vacuum setting given in the table is the trip point at which the quick-opening valve is opened. The vacuum tank had a volume of 0.125 cubic meters. Considering the connecting hoses as well as the pipe to be coated, the total volume varied from 0.221 cubic meters for 12.7 centimeter pipe down to 0.163 cubic meters for 8.9 centimeter pipe.

The flexible hose connecting the charging location to the pipe was approximately 3.8 centimeters inside diameter. It was estimated that the velocity in this line was maintained at approximately 20 meters per second with the venturi vacuum system being kept in operation.

Satisfactory coatings were obtained over a range of about 28°C from 140°C to 170°C. It is, however, required that the end-to-end pipe temperature not vary more than 5° to 8°C. Some experimentation is obviously required to achieve the optimum conditions for other coating materials and pipe sizes.

## Claims

1. A method for lining a heated tube (10) comprising: supporting the heated tube (10) to be internally coated; isolating a first end (14) of said tube (10) from the ingress of air, placing the tube interior in fluid communication (40) with a tank (34) via a second end (38) of said tube (10); establishing a preselected vacuum (50) in said tank (34) and said tube (10) by drawing air from a suction location (46) beyond said second end (38) of said tube (10); placing a charge (16) of coating material in an unpacked condition within a charged location (18) thereafter drawing the coating material into said tube (10) by suddenly placing said charged location (18) in fluid communication (20) with said tube (10), and following the flow of coating material with a flow of air, characterized by rotating said heated and horizontally supported tube (10); and drawing vacuum from a larger volume of said tank (34) than in said tube (10); said volume of said tank (34) being chosen so large relative to that of said tube (10), and the predetermined value of the vacuum therein so chosen that on sudden release of air into said tube (10) to be coated there is a sudden flow of air which is smoothly and immediately reduced to a lower vacuum level in the tube interior.

2. A method according to claim 1, characterized in that for placing the tube interior in fluid communication and establishing a vacuum said tank (34) is isolated from the ingress of air, a vacuum (50) is established in said tank (34) and thereafter said tube (10) is placed in fluid communication (44) with said tank (34).

3. A method according to claim 1 or 2, characterized in that for said charge (16) in fluid communication with said tube (10) said charge (16) is conveyed in said tube (10) at a first velocity thru said tube (10) at a lower velocity.

4. A method according to one of claims 1 to 3, characterized in that a charge (16) of coating material is measured, placing only said measured charge (16) within said charged location (18) which is open to atmosphere, and thereafter drawing substantially the entire charge (16) into said tube (10).

5. An apparatus for lining a heated tube (10) comprising: means (12) for supporting said heated tube (10); a container (18) for holding fusible particles which are to be delivered to said tube (10); a feedpipe (16) connected to said container (18) and sealably connectable to one end of said tube (10), an imperforate tank (34) having an inlet connection and an outlet connection; a discharge pipe (40) connectable to the second end of said tube (10) and connected to the inlet connection of said tank (34); a quick-opening valve (20) located in said feedpipe (16); a vacuum pump (46) connected to the outlet connection of said tank (34); sensing means (50) for sensing the level of vacuum within the heated tube; and means (70) for quickly opening said quick-opening valve (20) in response to said sensing means (50) when the measured vacuum level reaches a predetermined (72) vacuum level; characterized in that means (12) for horizontally supporting and rotating said tube (10) are provided; said tank (34) has a volume greater than said tube (10) and a plurality of supplementary tanks (60, 62); a plurality of pipes fluidly connected each of said supplementary tanks (60, 62) to said imperforate tank (34); and means for selectively isolating (64, 66) each of said supplementary tanks from said imperforate tank (34) are provided wherein the flow area of said feedpipe (16) is less than the flow area of said tube (10).

6. An apparatus according to claim 5, characterized by valve means (44) for isolating said imperforate tank (34) from said tube (10).

7. An apparatus according to claim 5 or 6, characterized by measuring means (26) for depositing in said container (18) only a predetermined quantity of fusible particles, said container (18) being open to atmosphere.

8. An apparatus according to one of claims 5 to 7, characterized by a dust collector (54) located downstream of said imperforate tank (34) and upstream of said vacuum pump (46).

## Patentansprüche

1. Verfahren zur Auskleidung eines erhitzten Rohres (10), bei dem das erhitzte Rohr (10) zur Innenbeschichtung abgestützt wird, ein erstes Ende (14) dieses Rohrs (10) gegen den Eintritt von Luft isoliert wird, der Rohrinnenraum über ein zweites Ende (38) dieses Rohrs (10) mit einem Behälter (34) in Fluidverbindung (40) gebracht wird, in diesem Behälter (34) und diesem Rohr (10) durch Absaugen von Luft an einer jenseits jenes zweiten Endes (38) dieses Rohrs (10) liegenden Saugstelle (46) ein vorbestimmtes Vakuum (50) erzeugt wird, ein Quantum (16) Beschichtungsmaterial in unverdichtetem Zustand in einen Ladebehälter (18) eingebracht und dann in dieses Rohr (10) eingesaugt wird, indem dieser Ladebehälter (18) plötzlich mit diesem Rohr (10) in Fluidverbindung (20) gebracht wird, und ein Luftstrom dem Strom Beschichtungsmaterial folgt, dadurch gekennzeichnet, dass dieses erhitzte und horizontal abgestützte Rohr (10) gedreht wird und ein grösseres Volumen in jenem Behälter (34) als in diesem Rohr (10) evakuiert wird, wobei dieses Volumen dieses Behälters (34) gegenüber dem Volumen dieses Rohrs (10) so gross und das vorbestimmte Ausmass des Vakuums darin so gewählt werden, dass bei plötzlichem Einlass von Luft in dieses zu beschichtende Rohr (10) ein plötzlicher Luftstrom entsteht, der sich gleichförmig und unmittelbar auf ein niedrigeres Vakuummass in dem Rohrinnenraum verringert.

2. Verfahren nach Anspruch 1, dadurch gekennzeichnet, dass zwecks Fluidverbindung mit dem Rohrinnenraum und Aufbau eines Vakuums, dieser Behälter (34) gegen Lufteintritt isoliert ist, darin ein Vakuum (50) erzeugt wird und danach dieses Rohr (10) in Fluidverbindung (44) mit diesem Behälter (34) gebracht wird.

3. Verfahren nach Anspruch 1 oder 2, dadurch gekennzeichnet, dass zwecks Fluidverbindung dieses Quantums (16) mit diesem Rohr (10), dieses Quantum (16) darin anfänglich mit einer niedrigeren Geschwindigkeit durch dieses Rohr (10) gefördet wird.

4. Verfahren nach einem der Ansprüche 1 bis 3, dadurch gekennzeichnet, dass ein Quantum (16) Beschichtungsmaterial abgemessen wird, nur dieses abgemessene Quantum (16) in jenen zur Atmosphäre offenen Ladebehälter (18) eingebracht wird und dann im wesentlichen das gesamte Quantum (16) in das Rohr (10) eingesaugt wird.

5. Vorrichtung zur Auskleidung eines erhitzen Rohrs (10), bestehend aud Mitteln (12) zur Abstützung dieses erhitzten Rohrs (10), einem Behälter (18) zur Aufnahme schmelzbarer, in dieses Rohr (10) zu fördernder Teilchen, einem Zufuhrrohr (16), das mit diesem Behälter (18) berbunden ist und dichtend mit einem Ende dieses Rohrs (10) verbunnden werden kann, einem Behälter (34) ohne Perforierungen und mit einer Einlass- und Auslassverbindung, einem Auslassrohr (40), das mit dem zweiten Ende dieses Rohrs (10) verbunden werden kann und mit der Einlassverbindung dieses Behälters (34) verbunden ist, einem in diesem Zufuhrrohr (16) angeordneten, schnell öffnenden Ventil (20), einer an die Auslassverbindung dieses Behälters (34) angeschlossenen Vakuumpumpe (46), Er^{f}assungsmittein (50) zur Erfassung des Vakuummasses im erhitzten Rohr und Mitteln (70) zum schnellen Oeffnen jenes schnell öffnenden Ventils (20) als Reaktion auf diese Erfassungsmittel (50), wenn das gemessene Vakuummass einen vorbestimmten (72) Vakuumwert erreicht, dadurch gekennzeichnet, dass Mittel (12) zur horizontalen Abstützung und Drehung dieses Rohrs (10) vorgesehen sind, dieser Behälter (34) ein grösseres Volumen als dieses Rohr (10) sowie mehrere Hilfsbehälters (60, 62) aufweist, mehrere Rohre dieser Hilfsbehälter (60, 62) jeweils mit diesem Behälter (34) ohne Perforierungen fluidverbunden sind, und Mittel zur wahlweisen Isolierung (64, 66) jedes dieser Hilfsbehälter von jenem Behälter (34) ohne Perforierungen vorgesehen sind, worin der Durchflussquerschnitt jenes Zufuhrrohrs (16) kleiner als der Durchflussquerschnitt dieses Rohrs (10) ist.

6. Vorrichtung nach Anspruch 5, gekennzeichnet durch Ventilmittel (44) zur Isolierung jenes Behälters (34) ohne Perforierungen von diesem Rohr (10).

7. Vorrichtung nach Anspruch 5 oder 6, gekennzeichnet durch Messeinrichtungen (26), damit nur eine vorbestimmte Menge schmelzbarer Teilchen in diesen Behälter (18) eingebracht wird, wobei dieser Behälter (18) zur Atmosphäre offen ist.

8. Vorrichtung nach einem der Ansprüche 5 bis 7, gekennzeichnet durch einen jenem Behälter (34) ohne Perforierungen nachgeschalteten und jener Vakuumpumpe (46) vorgeschalteten Staubabscheider (54).

## Revendications

1. Procédé pour revêtir un tube chauffé (10) comprenant le supportage du tube chauffé (10) à revêtir intérieurement, l'isolement d'une première extrémité (14) du dit tube (10) pour empêcher l'entrée de l'air, le raccordement (40) de l'intérieur du tube à un réservoir (34) par une seconde extrémité (38) du dit tube (10), l'établissement d'un vide prédéterminé (50) dans ledit réservoir (34) et ledit tube (10) en extrayant l'air par un orifice d'aspiration (46) àu-delà de ladite seconde extrémité (38) du dit tube (10), le placement d'une charge (16) de produit de revêtement à l'état non emballé en un endroit de chargement (18) et l'entraînement ultérieur du produit de revêtement dans ledit tube (10) en mettant ledit emplacement de chargement (18) en communication brusque (20) avec ledit tube (10) et en faisant suivre le débit de produit de revêtement par un débit d'air, caractérisé par le fait que le tube (10) chauffé et supporté horizontalement est mis en rotation, que le vide est établi dans ledit réservoir (40) ayant un volume supérieur à celui du dit tube (10), que ledit volume du dit réservoir (34) est choisi assez grand par rapport à celui du dit tube (10) et que le degré prédéterminé de vide dans celui-ci est choisi de façon à ce qu'une introduction soudaine d'air dans ledit tube (10) à revêtir provoque un débit d'air dans ledit tube (10) à revêtir provoque un débit d'air soudain qui est réduit doucement et immédiatement jusqu'à un degré de vide moins poussé à l'intérieur du tube.

2. Procédé selon la revendication 1, caractérisé en ce que, pour mettre l'intérieur du tube en communication et pour y faire le vide, ledit réservoir (34) est isolé pour empêcher l'entrée de l'air, que le vide (50) est établi dans ledit réservoir (34) et qu'ensuite ledit tube (10) est mis en communication (44) avec ledit réservoir (34).

3. Procédé selon la revendication 1 ou 2, caractérisé en ce que, lorsque ladite charge (16) étant en communication avec ledit tube (10), ladite charge (16) est transportée dans ledit tube (10) à une première vitesse à travers ledit tube (10) à une vitesse plus faible.

4. Procédé selon l'une des revendications 1 à 3, caractérisé en ce qu'une charge (16) de produit de revêtement est mesurée, que seule ladite charge mesurée (16) est placée au dit endroit de chargement (18) qui est en communication avec l'atmosphère et que la charge (16) est amenée ensuite presque entièrement dans ledit tube (10).

5. Appareil pour revêtir un tube chauffé (10), comprenant un dispositif (12) pour supporter ledit tube chauffé (10), un récipient (18) pour contenir des particules fusibles qui doivent être .amenées dans ledit tube (10), une tuyauterie d'alimentation (16) raccordée au dit récipient (18) et pouvant être raccordée d'une manière étanche à une extrémité du dit tube (10), un réservoir perforé (34) ayant un raccordement d'entrée et un raccordement de sortie, une tuyauterie d'évacuation (40) pouvant être raccordée à la seconde extrémité du dit tube (1µ) · et raccordée au raccordement d'entrée du dit reservoir (34), une vanne à ouverture rapide (20) disposée dans ladite tuyauterie d'alimentation (16), une pompe à vide (46) raccordée au raccordement de sortie du dit réservoir (34), un dispositif de détection (50) pour déterminer le degré de vide dans le tube chauffé et un dispositif (70) pour ouvrir rapidement ladite vanne à ouverture rapide (20) sous la commande du dit dispositif de détection (50) lorsque le degré de vide mesuré a atteint le degré de vide (72) prédéterminé, caractérisé en ce qu'il est prévu des dispositifs (12) pour supporter horizontalement et mettre en rotation ledit tube (10), que ledit réservoir (34) a un volume supérieur au dit tube (10) et à plusieurs réservoirs supplémentaires (60, 62), que plusieurs tuyauteries raccordent chacun des dits réservoirs supplémentaires (60, 62) au dit réservoir perforé (34) et qu'il est prévu des dispositifs pour assurer l'isolement sélectif (64, 66) de chacun des dits réservoirs supplémentaires par rapport au dit réservoir perforé (34), la section de passage de ladite tuyauterie d'alimentation (16) étant inférieure à la section de passage du dit tube (10).

6. Appareil selon la revendication 5, caractérisé par un dispositif à vanne (44) pour isoler ledit réservoir perforé (34) du dit tube (10).

7. Appareil selon la revendication 5 ou 6, caractérisé par un dispositif de mesure (26) pour déposer dans ledit récipient (18) seulement une quantité prédéterminée de particules fusibles, ledit récipient (18) étant en communication avec l'atmosphère.

8. Appareil selon l'une des revendications 5 à 7, caractérisé par un collecteur à poussières (54) disposé en aval du dit réservoir perforé (34) et en amont de ladite pompe à vide (46).
